

## UNITED STATES PATENT OFFICE.

148-21a5

ROBERT A. HADFIELD, OF SHEFFIELD, ENGLAND.

## GUN-HOUSE AND THE LIKE.

No. 863,063.

Specification of Letters Patent.

Patented Aug. 13, 1907.

Application filed October 18, 1906. Serial No. 339,542.

## To all whom it may concern:

Be it known that I, ROBERT A. HADFIELD, a subject of the King of Great Britain, and a resident of Sheffield, county of York, England, have invented an Improvement in Gun-Houses and the Like, of which the following description is a specification.

Gun houses and other similar structures designed for use on board war ships and in forts to withstand the attack of projectiles of various natures, are at present usually built up of a number of hard rolled or forged steel plates, such as Krupp cemented plates, suitably secured together by fastening devices such as bolts, keys or the like, these being driven in at great expense and even when so done they do not give a very satisfactory fastening. Such built-up structures are however open to various practical objections. They are very costly, owing to the mode of manufacture adopted in the formation of the plates with the necessary port and other holes, which have to be formed by machining or cutting out, and, owing to the mode of assembling and connecting the plates together, and to the shape of the plates adopted, (which, when rolled or forged, can only be bent or cambered with great difficulty and expense) they do not offer the most effective surface for resisting the action of projectiles but, on the contrary, are liable to receive by impact of heavy projectiles, concussive shocks of such magnitude as to cause fracture of the fastening devices and thereby displacement of the plates or even complete collapse of the whole structure.

Now the present invention has reference *inter alia* to gun houses made in one piece with the necessary port holes for guns, sighting and other purposes, and of such shape externally that projectiles on striking the same will be liable to be thrown off or deflected sidewise thereby in a more certain and effective manner than heretofore, whereby I am enabled to produce, at a comparatively moderate cost, gun houses better adapted to successfully withstand the attack of projectiles than gun houses of about similar thickness constructed as hereinbefore described. For this purpose, a gun house according to this invention is made in one piece of my improved or "Era" cast steel of dome or equivalent shape externally, that is to say of convex or rounded shape in all directions, and closed in all round, with the exception of the necessary holes or apertures for guns, sighting, and like purposes. For producing such a gun house, which may be of considerable weight, say for example one hundred tons or more, a mold is made of suitable composition such as fire resisting sand, or what is known as steel molding composition, dried in the usual way and having internally the formation of the intended finished gun house with one or more holes or apertures for one or more guns and for other purposes, and the gun house is formed by pouring into the mold so prepared, cast steel of such composition as will offer great resistance to penetration. For this purpose the

steel used should preferably be my special nickel chromium alloy steel low in carbon and free from or low in manganese, and technically termed "Era" steel. The carbon may vary from about 0.25% up to about .6%, the chromium from about 0.25% up to about 5.0% and the nickel from about 0.25% up to about 7.0%. Manganese, while preferably kept low, may go up to about 0.45%. Silicon and aluminium may be advantageously added separately or in conjunction for the purpose of producing sounder and better steel. The silicon should not usually exceed about 0.4%, ordinarily about 0.1% and aluminium up to about as high as 0.4% but ordinarily about 0.2%. Such steel can also advantageously be used for plates such as plain flat plates, deck plates, curved plates and other sections cast into form. Excellent steel for the purpose can be produced by melting in a cupola, ordinary hematite pig iron of good quality, running the molten metal into a converter, decarbonizing and desilicizing it, then adding, preferably in a molten or highly pre-heated condition, sufficient ferro-chromium and nickel to obtain steel of the following composition which is given as an example of manufacture: carbon about 0.35%, silicon about 0.12%, chromium about 1.7%, nickel about 3.3%, manganese about 0.35%, sulfur and phosphorus about 0.05% each.

The cast gun house is then preferably removed from the mold while hot and cooled down very slowly. Or the cooling may be arrested before it reaches atmospheric temperature so as to avoid any strains that might be brought about by afterwards reheating it from the cold. Or it may be submitted to a partial annealing treatment so that it will be in a sufficiently tough condition to allow of its being reduced to atmospheric temperature, when the casting is fettled or cleaned and, if desired, the heads or runners cut off. Its partial heat treatment may also consist in putting it into a temporarily hot annealing furnace and allowing it to cool down to about 300° C. The gun house is then, either when not previously cooled down at all, or when cooled down after the partial annealing treatment, submitted to the following special heat treatment. It is put into a furnace which is then heated to a high temperature, say between 900° C. and 1100° C. The gun house is then withdrawn from the furnace as soon as the requisite temperature has been reached and cooled in the open air. Where the greatest possible toughness is required, it is necessary, in order to get the best results, to withdraw the gun house from the furnace as stated, and cool it in such a manner that its rate of cooling will proceed more quickly than if it be left in the furnace. The cooling may, of course, be effected in the furnace if desired, but cooling in the external air is preferred. The heads or risers are then removed, if this has not already been done. The gun house is then heated to from 700° C. to 850° C., usually

preferring about 760° C., and cooled down as far as desired, say to about 640° C., either slowly in the furnace or it may be air cooled, then reheated to between 700° C. and 850° C., and cooled to between 640° C. and 690° C., and wholly or partially quenched in water, due care being taken that it is not allowed to remain too long in the water to produce a greater degree of hardness or stiffness than required. The gun house is then again heated to between 570° C. and 640° C., the preferable temperature depending upon the particular composition of the steel used, and allowed to cool in the furnace. It is then reheated to between 570° C. and 640° C. and quenched outright, preferably in water. In this way a gun house of very high efficiency in resisting gun fire can be produced.

If it is desired to render a gun house such as described hard on its outer surface, it is suitably carbonized where required. For this purpose the cast gun house is put into a furnace and upon its surface a suitable carbonizing medium, for example carbon is placed. The furnace is then raised to a high temperature, say between 900° C. and 1100° C. and the gun house allowed to remain therein for several days, the actual period depending upon the extent to which the carbonizing is to be carried. The gun house is then allowed to cool gradually down. This is usually done in the furnace, but may be done in the open air, though the latter method is chiefly preferable for non-carbonized articles. After this treatment, the heads or risers are removed and the gun house subjected to the heat treatment hereinbefore described, commencing in heating it to 700° C. to 850° C. In this case, after the final quenching outright of the gun house in water or other cooling medium, it is taper heated, that is to say, it is heated so that the face or outer side assumes a temperature of from 700° C. to 770° C., tapering to a temperature at the inner side of from 400° C. to 600° C., whereupon the gun house is dipped in or sprayed with oil or water, according to the hardness required, so that the outer side, being hotter than the inner side, will become hard while the inner side remains soft and tough. In some cases, as for example when a very soft steel is used, that is to say, one low in carbon, a uniform instead of a "taper" heating may be adopted for the face hardening treatment.

Owing to the disposition of the material and its extraordinary toughness and tenacity, as compared with mild steel, most excellent results are obtained by the treatment first described without its being necessary to carbonize or make hard the face of the article.

Gun houses designed for use in land forts, as well as on war ships, manifestly can be constructed in the manner described.

Director towers, roofs, glacis plates, communication tubes, ammunition tubes, and other similar articles used on war ships, may also, according to the present invention, be manufactured in the manner and of like material to that hereinbefore described with reference to gun houses. The towers will preferably be of oval or like shape in horizontal section and of upwardly tapering shape with a rounded or convex roof or head, so as nowhere to present a flat surface for attack of projectiles but any suitable shape can be employed.

The construction of gun houses and other protective structures of cast steel having such a composition as hereinbefore set forth and treated as described is of great advantage owing to equal strength and toughness effected in all directions of the structure.

Wrought steel varies in strength and toughness according to the way in which it is forged, hammered or rolled, but the steel described herein and treated as set forth has equal strength and toughness in all directions, whether longitudinal or transverse.

In all cases, the fact of being able to produce by my invention, a material of the desired composition and quality, makes it possible to dispose and apply cast products in such a way as enables the naval architect to introduce forms and shapes that would otherwise be impracticable, and which in ordinary steel, even if cast, would not be of sufficient practical value to permit of their employment on war and other ships.

Having described my invention, what I claim as new and desire to secure by Letters Patent is:

1. As a new article of manufacture, a gun house or the like formed of nickel chromium steel cast as an integral structure of the form in which it is to be used, heated to a temperature of between 900° C. and 1100° C., and thereafter cooled in the air, then heated to a lower temperature, and finally quenched in a cooling liquid.

2. As a new article of manufacture, a gun house or the like formed of nickel chromium steel cast as an integral structure of the form in which it is to be used, the casting being slowly cooled down to a temperature above that of the atmosphere, heated to a predetermined high temperature and slowly cooled, reheated to a lower temperature, and finally cooled by quenching.

3. As a new article of manufacture, a gun house or the like formed of nickel chromium steel cast as an integral structure of the form in which it is to be used, the casting being slowly cooled down to about 300° C., then heated to a temperature of between 900° C. and 1100° C. and slowly cooled, reheated to a lower temperature, and finally quenched in a cooling liquid.

In testimony whereof, I have signed my name to this specification, in the presence of two subscribing witnesses.

ROBERT A. HADFIELD.

Witnesses:

CHAS. N. DANIELS,  
LUTHER J. PARR.